

## UNITED STATES PATENT OFFICE.

HERBERT C. BUGBIRD, OF RICHMOND, NEW YORK.

## METHOD AND MEANS FOR PREPARING EXPLOSIVES, AND RESULTING EXPLOSIVES.

No Drawing. Application filed May 2, 1925, Serial No. 27,345. Renewed August 7, 1928.

My present invention relates to methods of fabricating absorbents for liquid oxygen for use as explosives, and particularly to carbonaceous absorbents derived from the lignin 5 liquors or residues obtained in the manufacture of wood pulp by the alkali (soda) or other suitable process, but particularly by the alkali (soda) process, and aims to devise methods of the general character specified which are simple to practice, easy, economical and convenient to carry out, requiring simple apparatus and few manipulations for this purpose, and which result in a superior product for the intended purpose, this 15 product, which also comprises a part of the present invention, being characterized by its high density, its high degree of absorptiveness for liquid oxygen, its high degree of retentiveness for the absorbed liquid oxygen, 20 and its high degree of combustibility, all desirable properties for the intended purpose. My invention includes also the resulting explosive and cartridge containing the same, and involves other advantages in manipulation, use and superiorities of the process and resulting product which will in part be pointed out hereinafter and which will in part be obvious to those skilled in the art to which the present invention relates.

In the accompanying specification I shall describe an illustrative embodiment of the method of the present invention. In the accompanying specification I shall also describe illustrative embodiments of the products of the present invention, particularly the products resulting from the practice of the aforesaid illustrative embodiment of the method of the present invention. It is, however, to be clearly understood that my invention is not limited to the specific embodiments thereof herein described for purposes of illustration only. It is further to be understood that the process is not limited to the production of the specific products herein described by way of illustration merely, and that the products may be made by other embodiments of the process than that herein specifically described for purposes of example merely.

Referring to the aforesaid illustrative embodiments of the present invention, and particularly to the aforesaid illustrative embodiment of the method, I prefer to use as the raw material for the fabrication of the product of the present invention liquors rich in dissolved lignin, preferably such liquors de-

rived from the manufacture of wood pulp by the alkali (soda) process, especially where wood pulp is derived from woods, such as spruce, pine and the like, rich in resins or other forms of lignin. Such liquors are particularly desirable, since they yield a high purity carbon characterized by high density and great absorptiveness and retentiveness for liquid oxygen, as hereinafter described in considerable detail.

These liquors are now carbonized, preferably with controlled access of air or even with the total exclusion of air. This is done in order to prevent too great combustion and consequent loss of carbon values in the final material. Preferably such carbonization takes place in retorts which are sealed against the ingress of air or to which air is admitted in very small amounts only to carry off by combustion or otherwise more volatile carbonaceous materials to thus leave a very open or porous carbonized lignin residue in the retort.

The carbonized lignin residues thus obtained will be found to be in a granular condition, the grains of which vary in size to a considerable degree and are quite uneven in size. The material also will be found to contain in the pores thereof a considerable amount, often as high as ten (10) per cent, of alkaline carbonates, particularly sodium carbonate, where the pulp has been made by the soda process, together with other mineral substances. The carbonized lignin residues thus obtained are now thoroughly leached, first with water, to remove water-soluble mineral substances, and thereafter, if desired, although this step may be omitted, with acidulated water, such as water acidulated with about one-half to one per cent of hydrochloric acid, to remove acid-soluble mineral substances. The purpose of this treatment or treatments is to reduce to a minimum the mineral constituents of the carbon so as to obtain a carbon characterized by maximum combustibility.

I now take the leached carbonized lignin residues, whether or not the same have been previously subjected to the acid treatment specified above, and submit the same to a slight grinding action to reduce the grains to a more or less uniform size so that the largest grains are not more than about one-quarter of an inch in their longest dimension and so that not more than about twenty-five per cent

60  
6570  
75

80

85  
90

95

100

105

110

of the material will pass through a one hundred mesh screen. Care should be taken during this slight grinding action, the purpose of which is to obtain a more uniform, even-sized material which is very suitable for use in smaller sized cartridges, to see that the material is not too finely ground, which would convert it from a highly absorptive material for liquid oxygen, suitable for the purposes of the present invention, into a material characterized by considerable decolorizing power but a low degree of absorptiveness for liquid oxygen, which would make the material unfit for the purposes of the present invention.

I have found that in general the density of the material when poured as freely into a container as it would be into the cartridge wrapper, should be not less than about 0.20. I have also found that the degree of absorptiveness of the material for liquid oxygen should be not less than about 2.6 times its own weight, and preferably about 3.0 times its own weight, or even over, so as to be suitable for use under actual field conditions and to take care of any liquid oxygen that might be evaporated up to the time that the cartridge is actually exploded.

It may here be stated, that by carefully controlling the carbonization of the lignin liquors or residues in the retorts, grains of the proper size may be and often are obtained without any grinding action whatsoever. In any event, the grinding action should be carefully controlled and regulated to yield a carbon characterized by a high degree of absorptiveness and a comparatively low degree of decolorizing power, rather than a low degree of absorptiveness and a high degree of decolorizing power. I have found that the properties of absorptiveness and decolorizing power vary generally in approximately inverse proportion, absorptiveness depending on a comparatively large grain and being characterized by a comparatively low degree of decolorizing power, decolorizing power being apparently dependent upon small grains of a low degree of absorptiveness.

The material obtained as above described may now be packed into suitable cartridge containers. I prefer to use a container which is completely and readily combustible and which has proper insulating properties to prevent too ready absorption of heat with consequent evaporation of the liquid oxygen. For this purpose I prefer to use a cartridge container which has a cotton fibre base, such as certain red fibre papers which may be readily obtained in the open market. This paper may readily be formed into containers of the desired size which are then packed with the granular leached carbonized lignin residues obtained as above described, after which the liquid oxygen is added, the car-

tridge sealed, stored and finally put in place, and exploded by a percussion cap or otherwise.

The material obtained as above described is characterized by its high density, its uniformity, its high degree of absorptiveness and its correspondingly high degree of retentiveness for the liquid oxygen, making it ideally suited for use under actual field conditions for blasting and similar purposes. Actual tests show that this material is ideally suited for the purpose and is at the same time quite cheap and may therefore be readily and economically manufactured in large quantities for the intended purpose. The process as described above is very simple to practice, makes use of an otherwise waste material, and requires very simple apparatus and few manipulations for its successful practice. The absorbent itself possesses the many advantages already specified above, and the resulting explosive and cartridges containing the same are further characterized by their cheapness, the ease with which they may be prepared, and their remarkable efficiency in use under actual field conditions. Other advantages of the present invention will readily occur to those skilled in the art to which the same relates.

What I claim as my invention is:

1. The method of preparing granular carbonized lignin residues for use as an absorbent for liquid oxygen, which comprises leaching said material to substantial freedom from water-soluble mineral matters to reduce the proportion of incombustible constituents of said material to a minimum and reducing the grains of the carbonized material to such a size that their density will be at least equal to about 0.20 and their degree of absorptiveness for liquid oxygen at least equal to 2.6 times their own weight.

2. The method of preparing granular carbonized lignin residues for use as an absorbent for liquid oxygen, which comprises leaching said material with an acid solution to substantial freedom from water-soluble and acid-soluble mineral matters to reduce the proportion of incombustible constituents of said material to a minimum and reducing the grains of the carbonized material to such a size that their density will be at least equal to about 0.20 and their degree of absorptiveness for liquid oxygen at least equal to 2.6 times their own weight.

3. The method of preparing granular carbonized lignin residues for use as an absorbent for liquid oxygen, which comprises leaching said material to substantial freedom from water-soluble mineral matters to reduce the proportion of incombustible constituents of said material to a minimum and reducing the grains of the carbonized material to such a size that their density will be at least equal to about 0.20 and their degree

of absorptiveness for liquid oxygen at least equal to 3.0 times their own weight.

4. The method of preparing granular carbonized lignin residues for use as an absorbent for liquid oxygen, which comprises leaching said material with an acid solution to substantial freedom from water-soluble and acid-soluble mineral matters to reduce the proportion of incombustible constituents of said material to a minimum and reducing the grains of the carbonized material to such a size that their density will be at least equal to about 0.20 and their degree of absorptiveness for liquid oxygen at least equal to 3.0 times their own weight.

5. The method of preparing granular carbonized lignin residues for use as an absorbent for liquid oxygen, which comprises leaching said material with an acid solution to substantial freedom from water-soluble and acid-soluble mineral matters to reduce the proportion of incombustible constituents of said material to a minimum and reducing the grains of the carbonized material to such a size that not more than twenty-five (25) per cent of the material will pass through a one hundred mesh screen and their density will be at least equal to about 0.20 and their degree of absorptiveness for liquid oxygen at least equal to 3.0 times their own weight.

6. The method of preparing granular carbonized lignin residues for use as an absorbent for liquid oxygen, which comprises leaching said material with an acid solution to substantial freedom from water-soluble and acid-soluble mineral matters to reduce the proportion of incombustible constituents of said material to a minimum and reducing the grains of the carbonized material to such a size that not more than twenty-five (25) per cent of the material will pass through a one hundred mesh screen and their density will be at least equal to about 0.20 and their degree of absorptiveness for liquid oxygen at least equal to 2.6 times their own weight.

7. The method of preparing granular carbonized lignin residues for use as an absorbent for liquid oxygen, which comprises leaching said material to substantial freedom from water-soluble mineral matters to reduce the proportion of incombustible constituents of said material to a minimum and reducing the grains of the carbonized material to such a size that not more than twenty-five (25) per cent of the material will pass through a one hundred mesh screen and their density will be at least equal to about 0.20 and their degree of absorptiveness for liquid oxygen at least equal to 3.0 times their own weight.

8. The method of preparing granular carbonized lignin residues for use as an absorbent for liquid oxygen, which comprises leaching said material to substantial freedom from water-soluble mineral matters to

reduce the proportion of incombustible constituents of said material to a minimum and reducing the grains of the carbonized material to such a size that not more than twenty-five (25) per cent of the material will pass through a one hundred mesh screen and their density will be at least equal to about 0.20 and their degree of absorptiveness for liquid oxygen at least equal to 2.6 times their own weight.

9. The method of preparing carbonaceous material for use as an absorbent for liquid oxygen for use as an explosive, which comprises carbonizing liquors rich in dissolved lignin material with controlled access of air to form a granular carbonized lignin residue, and thereafter leaching said material with an acid solution to substantial freedom from water-soluble and acid-soluble mineral matters to reduce the proportion of incombustible constituents of said material to a minimum and reducing the grains of the carbonized material to such a size that their density will be at least equal to about 0.20 and their degree of absorptiveness for liquid oxygen at least equal to 3.0 times their own weight.

10. The method of preparing carbonaceous material for use as an absorbent for liquid oxygen for use as an explosive, which comprises carbonizing liquors rich in dissolved lignin material with controlled access of air to form a granular carbonized lignin residue, and thereafter leaching said material with an acid solution to substantial freedom from water-soluble and acid-soluble mineral matters to reduce the proportion of incombustible constituents of said material to a minimum and reducing the grains of the carbonized material to such a size that their density will be at least equal to about 0.20 and their degree of absorptiveness for liquid oxygen at least equal to 2.6 times their own weight.

11. The method of preparing carbonaceous material for use as an absorbent for liquid oxygen for use as an explosive, which comprises carbonizing liquors rich in dissolved lignin material with controlled access of air to form a granular carbonized lignin residue, and thereafter leaching said material to substantial freedom from water-soluble mineral matters to reduce the proportion of incombustible constituents of said material to a minimum and reducing the grains of the carbonized material to such a size that their density will be at least equal to about 0.20 and their degree of absorptiveness for liquid oxygen at least equal to 3.0 times their own weight.

12. The method of preparing carbonaceous material for use as an absorbent for liquid oxygen for use as an explosive, which comprises carbonizing liquors rich in dissolved lignin material with controlled access

of air to form a granular carbonized lignin residue, and thereafter leaching said material to substantial freedom from water-soluble mineral matters to reduce the proportion of incombustible constituents of said material to a minimum and reducing the grains of the carbonized material to such a size that their density will be at least equal to about 0.20 and their degree of absorptiveness for liquid oxygen at least equal to 2.6 times their own weight.

13. An absorbent for liquid oxygen for use as an explosive, comprising granular carbonized lignin residues substantially free from water-soluble mineral matters and having a minimum proportion of incombustible constituents, the density of the material being at least equal to about 0.20 and the degree of absorptiveness of the material for liquid oxygen being at least equal to 2.6 times its own weight.

14. An absorbent for liquid oxygen for use as an explosive, comprising granular carbonized lignin residues substantially free from water-soluble and acid-soluble mineral matters and having a minimum proportion of incombustible constituents, the density of the material being at least equal to about 0.20 and the degree of absorptiveness of the material for liquid oxygen being at least equal to 2.6 times its own weight.

15. An absorbent for liquid oxygen for use as an explosive, comprising granular carbonized lignin residues substantially free from water-soluble mineral matters and having a minimum proportion of incombustible constituents, the density of the material being at least equal to about 0.20 and the degree of absorptiveness of the material for liquid oxygen being at least equal to 3.0 times its own weight.

16. An absorbent for liquid oxygen for use as an explosive, comprising granular carbonized lignin residues substantially free from water-soluble and acid-soluble mineral matters and having a minimum proportion of incombustible constituents, the density of the material being at least equal to about 0.20 and the degree of absorptiveness of the material for liquid oxygen being at least equal to 3.0 times its own weight.

17. An absorbent for liquid oxygen for use as an explosive, comprising granular carbonized lignin residues substantially free from water-soluble and acid-soluble mineral matters and having a minimum proportion of incombustible constituents, the grains of the material being of such a size that not more than twenty-five (25) per cent of the material will pass through a one hundred mesh screen.

18. An absorbent for liquid oxygen for use as an explosive, comprising granular carbonized lignin residues substantially free from water-soluble mineral matters and

having a minimum proportion of incombustible constituents, the grains of the material being of such a size that not more than twenty-five (25) per cent of the material will pass through a one hundred mesh screen.

19. An absorbent for liquid oxygen for use as an explosive, comprising granular carbonized lignin residues substantially free from water-soluble and acid-soluble mineral matters and having a minimum proportion of incombustible constituents, the density of the material being at least equal to about 0.20 and the degree of absorptiveness of the material for liquid oxygen being at least equal to 2.6 times its own weight, the grains of the material being of such a size that not more than twenty-five (25) per cent of the material will pass through a one hundred mesh screen.

20. An absorbent for liquid oxygen for use as an explosive, comprising granular carbonized lignin residues substantially free from water-soluble mineral matters and having a minimum proportion of incombustible constituents, the density of the material being at least equal to about 0.20 and the degree of absorptiveness of the material for liquid oxygen being at least equal to 2.6 times its own weight, the grains of the material being of such a size that not more than twenty-five (25) per cent of the material will pass through a one hundred mesh screen.

21. A cartridge comprising a combustible container charged with an explosive comprising an absorbent for liquid oxygen for use as an explosive, comprising granular carbonized lignin residues substantially free from water-soluble and acid-soluble mineral matters and having a minimum proportion of incombustible constituents, the density of the material being at least equal to about 0.20 and the degree of absorptiveness of the material for liquid oxygen being at least equal to 2.6 times its own weight, the grains of the material being of such a size that not more than twenty-five (25) per cent of the material will pass through a one hundred mesh screen, said absorbent containing absorbed therein an amount of liquid oxygen sufficient for complete combustion of the absorbent under actual field conditions and allowing for average evaporation of liquid oxygen.

22. A cartridge comprising a combustible container charged with an explosive comprising an absorbent for liquid oxygen for use as an explosive, comprising granular carbonized lignin residues substantially free from water-soluble and acid-soluble mineral matters and having a minimum proportion of incombustible constituents, the grains of the material being of such a size that not more than twenty-five (25) per cent of the

material will pass through a one hundred mesh screen, said absorbent containing absorbed therein an amount of liquid oxygen sufficient for complete combustion of the absorbent under actual field conditions and allowing for average evaporation of liquid oxygen.

23. A cartridge comprising a combustible container charged with an explosive comprising an absorbent for liquid oxygen for use as an explosive, comprising granular carbonized lignin residues substantially free from water-soluble mineral matters and having a minimum proportion of incombustible constituents, the density of the material being at least equal to about 0.20 and the degree of absorptiveness of the material for liquid oxygen being at least equal to 3.0 times its own weight, said absorbent containing absorbed therein an amount of liquid oxygen sufficient for complete combustion of the absorbent under actual field conditions and allowing for average evaporation of liquid oxygen.

24. A cartridge comprising a combustible container charged with an explosive comprising an absorbent for liquid oxygen for use as an explosive, comprising granular carbonized lignin residues substantially free from water-soluble mineral matters and having a minimum proportion of incombustible constituents, the density of the material being at least equal to about 0.20 and the degree of absorptiveness of the material for liquid oxygen being at least equal to 2.6 times its own weight, said absorbent containing absorbed therein an amount of liquid oxygen sufficient for complete combustion of the absorbent under actual field conditions and allowing for average evaporation of liquid oxygen.

25. A cartridge comprising a combustible container charged with an explosive comprising an absorbent for liquid oxygen for use as an explosive, comprising granular carbonized lignin residues substantially free from water-soluble mineral matters and having a minimum proportion of incombustible constituents, said absorbent containing absorbed therein an amount of liquid oxygen sufficient for complete combustion of the absorbent under actual field conditions and allowing for average evaporation of liquid oxygen.

26. A cartridge comprising a combustible container charged with an explosive comprising an absorbent for liquid oxygen for use as an explosive, comprising granular carbonized lignin residues substantially free from water-soluble mineral matters and having a minimum proportion of incombustible constituents, the density of the material being at least equal to about 0.20 and the degree of absorptiveness of the mate-

rial for liquid oxygen being at least equal to 2.6 times its own weight, the grains of the material being of such a size that not more than twenty-five (25) per cent of the material will pass through a one hundred mesh screen, said absorbent containing absorbed therein an amount of liquid oxygen sufficient for complete combustion of the absorbent under actual field conditions and allowing for average evaporation of liquid oxygen.

27. A cartridge comprising a combustible container charged with an explosive comprising an absorbent for liquid oxygen for use as an explosive, comprising granular carbonized lignin residues substantially free from water-soluble mineral matters and having a minimum proportion of incombustible constituents, the grains of the material being of such size that not more than twenty-five (25) per cent of the material will pass through a one hundred mesh screen, said absorbent containing absorbed therein an amount of liquid oxygen sufficient for complete combustion of the absorbent under actual field conditions and allowing for average evaporation of liquid oxygen.

28. A cartridge comprising a combustible container charged with an explosive comprising an absorbent for liquid oxygen for use as an explosive, comprising granular carbonized lignin residues substantially free from water-soluble and acid-soluble mineral matters and having a minimum proportion of incombustible constituents, the density of the material being at least equal to about 0.20 and the degree of absorptiveness of the material for liquid oxygen being at least equal to 3.0 times its own weight, said absorbent containing absorbed therein an amount of liquid oxygen sufficient for complete combustion of the absorbent under actual field conditions and allowing for average evaporation of liquid oxygen.

29. A cartridge comprising a combustible container charged with an explosive comprising an absorbent for liquid oxygen for use as an explosive, comprising granular carbonized lignin residues substantially free from water-soluble and acid-soluble mineral matters and having a minimum proportion of incombustible constituents, the density of the material being at least equal to about 0.20 and the degree of absorptiveness of the material for liquid oxygen being at least equal to 2.6 times its own weight, said absorbent containing absorbed therein an amount of liquid oxygen sufficient for complete combustion of the absorbent under actual field conditions and allowing for average evaporation of liquid oxygen.

30. A cartridge comprising a combustible container charged with an explosive comprising an absorbent for liquid oxygen for

use as an explosive, comprising granular carbonized lignin residues substantially free from water-soluble and acid-soluble mineral matters and having a minimum proportion of incombustible constituents, said absorbent containing absorbed therein an amount of liquid oxygen sufficient for complete com-

bustion of the absorbent under actual field conditions and allowing for average evaporation of liquid oxygen.

In testimony whereof, I have signed my name to this specification this 8th day of April, 1925.

HERBERT C. BUGBIRD.